

# United States Patent Office

2,750,306

Patented June 12, 1956

1

2,750,306

## TREATMENT OF TEXTILE MATERIALS WITH QUATERNARY AMMONIUM COMPOUNDS

Raymond A. Pingree, Cranston, and Chester U. Stevens, Saylesville, R. I., assignors to Crown Chemical Corporation, Providence, R. I., a corporation of Rhode Island

No Drawing. Application June 24, 1954,  
Serial No. 439,128

8 Claims. (Cl. 117—121)

This invention relates to the treatment of textile materials including fabrics, yarns and threads whereby there is imparted thereto permanent water-repellent characteristics. The fibers of the textile to which this property can be conferred include cellulosic (cotton, linen, regenerated cellulose rayons, etc.), protein (wool "Vicara," silk), cellulose esters (acetate rayon), polyamide fibers (nylon), acrylic type ("Acrilan," "Orlon," "Dyne") and polyester type ("Dacron").<sup>1</sup>

It is an object of the present invention to provide an improved process for imparting a high degree of water-repellency to any of the aforesaid types of textile fibers, and which property is not seriously reduced by repeated launderings and/or dry cleanings wherein conventional solvents are employed in these two distinctly different cleaning operations.

It is a further object of this invention to provide an improved process for imparting a high degree of water-repellency to the various types of textile fibers without causing fiber degradation.

Other and further important objects of this invention will become apparent from reading the description below.

In British Patent No. 477,991, granted to Baldwin, Evans and Salkeld and their assignees, there is described a process for treating cellulosic materials in aqueous solution with a compound of the general formula



whereby there is imparted to the fibers water-repellent properties. In that formula R stands for the alkyl radical of a long chain fatty acid, N(tert) stands for a molecule of a tertiary base, such as pyridine, quinoline or trimethyl amine, while X stands for a monovalent acid group, such as Cl. Some of the specific treating agents in this patent are stearamidomethylpyridinium sulfate or chloride and laurylamidomethylpyridinium chloride. However, the process of this patent using these compounds will not impart a sufficiently high degree of initial and durable water repellency nor will the treated textile materials withstand laundering and dry cleaning to the high degree required to meet the more recent Government and civilian specifications.

We have found that the above objects of the present invention can be accomplished by treating the textile fibers with an aqueous bath of a new, water-dispersible quaternary ammonium compound presently to be described, squeezing the fibers to remove surplus liquid, drying to remove most of the moisture left therein, and finally subjecting to an elevated temperature to form the water-repellent residue on the fibers. As pointed out in

2

the initial paragraph, the imparting of a high degree of water-repellency is not confined to natural or regenerated cellulosic fibers but embraces the protein and cellulose ester types and the more recently discovered synthetic types mentioned herein.

Satisfactory water-repellent characteristic can be conferred to the fabric by depositing on the fabric 1.0 to 4.0% of these quaternary ammonium compounds.

The compounds which we employ for the purpose of this invention are in themselves novel compounds and are more fully described and claimed in our copending patent application Serial No. 439,127 of even date here-with. Briefly stated, the synthesis of these compounds, which are water-dispersible quaternary ammonium compounds, the structural formula of which has not been established, is as follows: a chloromethyl acyl amide of the general formula  $\text{R}.\text{CONH}.\text{CH}_2\text{X}$ , where R is a paraffin hydrocarbon radical and the acyl group has a chain length of 10 to 22 carbon atoms inclusive and X is chlorine, is reacted with a straight chain alkyl nitrile whose alkyl group has a length of 10 to 22 carbon atoms inclusive; this resulting compound is treated with formaldehyde and hydrogen chloride to form a chloromethyl derivative of this first intermediate; and this second intermediate is then reacted with either pyridine or the C-alkyl substituted pyridines to form the water-dispersible quaternary ammonium compounds. The steps of the reaction, particularly the first two steps, are preferably carried out in the presence of an inert, volatile organic solvent for the reactants such as benzene, dioxane, ethylene dichloride, isohexane or ethyl acetate, which solvents prevent the mass from solidifying during the process, thus facilitating handling and control. In place of hydrochloric acid other compounds of chlorine capable of releasing HCl, such as  $\text{PCl}_3$ ,  $\text{PCl}_5$ ,  $\text{SOCl}_2$  may be used. Furthermore, as explained in that invention, those new, water-dispersible quaternary ammonium compounds can be prepared by other alternative procedures. Formaldehyde is preferably used in a polymeric form, as paraformaldehyde. The substituted pyridines include all the isomers of picoline, lutidine, collidine and such disubstituted specific compounds as 2-methyl-5-ethyl pyridine.

We have not been able to establish proof of the structure of the compounds formed in our process. We believe, however, that the reaction between the alkyl nitrile and the chloromethylacylamide does proceed to form an imino chloride, thus:



and that the chloromethylation of the imino chloride proceeds:



60 The final quaternary compound would be:



65 The advantages which our process of treating textile materials possesses over the British Patent No. 477,991 referred to previously reside in the fact that the water-repellent effect is more durable to laundering.

70 Suitable proportions in preparing the quaternary ammonium compounds which are the treating agents of the present invention and the intermediates in the syn-

<sup>1</sup> "Vicara" is a trademark of the Virginia-Carolina Chemical Co. of Richmond, Virginia, for wool-like fiber. "Acrilan" is a trademark of Chemstrand Corp., Decatur, Ala., for acrylic textile fiber. "Orlon" is a trademark of E. I. du Pont de Nemours Co., Inc. of Wilmington, Delaware, for acrylic fiber yarn and staple. "Dyne" is a trademark of Union Carbide and Carbon Company of New York City for acrylic fiber. "Dacron" is a trademark of E. I. du Pont de Nemours Co., Inc. of Wilmington, Delaware, for polyester fiber yarn and staple.

thesis thereof are 1 mol equivalent of the chloromethyl acyl amide, approximately 0.5-1.5 mol equivalents of the straight chain alkyl nitrile, approximately 0.5-1.5 mol equivalents of formaldehyde and 0.5-1.5 mol equivalents of a chlorinating agent which may be hydrogen chloride or others mentioned herein, and approximately 0.5-1.5 mol equivalents of a tertiary amine from the group consisting of pyridine and C-alkyl substituted pyridines.

Preferred temperature range for the reaction between the chloromethyl acyl amide and the alkyl nitriles, and also for the chloromethylation of this intermediate with formaldehyde and hydrogen chloride is 60° to 75° C. inclusive. Formation of the final product, the pyridinium compound, takes place readily at temperatures of 50° to 75° C. inclusive. No advantage has been observed by conducting these reactions at any specific temperatures within the limits stated. These temperatures should not be considered as critical. Below the lowest temperatures the mentioned supra speed of reaction tends to slacken. Generally speaking, temperatures above the highest in these ranges offer no advantage in yield, and increase of temperature entails a costlier condition of operation. The reaction temperature necessary to give optimum yields varies with the reactants and proportions.

It will be understood that the acyl amido methyl chloride reactant need not be that of one fatty acid, since mixtures of two or more of the general formula



where R denotes a paraffin hydrocarbon and X a halogen, may be employed. And mixtures of the other reactants, to wit, the alkyl nitrile and the tertiary amine, etc., may be employed. To confer latitude in properties this may be desirable.

Those water-dispersible quaternary ammonium compounds, which are formed from paraffin organic acid amides and alkyl nitriles, the amide of which former specified reactant is substituted by chloromethyl, each of which reactants has a chain length of 16 carbon atoms and above up to and including 22 carbon atoms, are preferred. Specific members of these amides are: chloromethyl stearamide (stearyl amido methyl chloride), chloromethyl palmitamide (palmityl amido methyl chloride) and chloromethyl lauramide (lauryl amido methyl chloride). Specific alkyl nitriles are: lauromonitrile (dodecane nitrile), myristonitrile (tetradecane nitrile), palmononitrile (hexadecane nitrile), stearononitrile (octadecane nitrile), and cerotononitrile (hexacosane nitrile). As the chain length of the acid amide and the alkyl nitrile falls below C<sub>16</sub> the water-repellency diminishes.

Unsaturated hydrocarbon acid amides and nitriles may be tolerated in mixtures with the fully saturated compounds. Commercial amides and nitriles containing up to 5% of oleic acid derivatives have been successfully used in the process. Appreciably higher percentages of the unsaturated hydrocarbon compounds cause a serious loss of water repellency in the performance of the resulting quaternary ammonium compounds.

In applying these quaternary ammonium compounds to textiles, the temperature of the aqueous treating bath or solution should preferably not be higher than 50° C., inasmuch as higher temperatures may cause premature decomposition of the quaternary ammonium treating agent. In the drying step which follows in its sequence the squeezing step, the treated moist textile may be dried at conventional drying temperatures (100°-150° C.). Decomposition of the impregnating agent on the textile material, which in practice is termed "curing," to form a water-repellent residue thereon, is a function of time v. temperature. It may be accomplished in about two minutes at 150° C., which is about a practical minimum temperature, or at the other extreme, i. e., upper temperature range, in about thirty seconds at 230° C., which is about a practical maximum temperature. In between these temperatures the time will vary inversely with the

temperature, there being a corresponding decrease in time with the rise in temperature.

During the baking step hydrochloric acid is liberated in the decomposition of the quaternary ammonium compound. This will cause serious damage to the fiber in the nature of its being somewhat tendered, i. e., its tensile strength is diminished; this is believed to be due to contact of the fiber with free hot hydrochloric acid. By including in the treating liquid an agent capable of neutralization, this destructive action is eliminated. Suitable water-soluble, neutralizing agents are the salts of strong bases and weak acids such as the sodium or potassium salts of acetic or lactic acids. These salts are incorporated in the aqueous treating bath in an amount sufficient to prevent fiber degradation, commonly termed tenderizing.

Without limiting our invention to any particular procedure, the following examples will serve to illustrate our preferred mode of operation.

#### EXAMPLE I

##### A. Preparation of the quaternary ammonium compound

Three hundred thirteen (313) grams of methylol stearamide is mixed with six hundred (600) grams of benzene to form a slurry. While agitating vigorously and maintaining the temperature at 40° to 60° C., forty (40) grams of hydrogen chloride gas is slowly bubbled beneath the surface. Stirring is continued for 10 minutes after the hydrogen chloride has been added.

To the chloromethyl stearamide (stearyl amido methyl chloride) thus formed is added two hundred sixty-five (265) grams of octadecane nitrile (stearonitrile). The temperature is raised to 65° to 70° C. and stirring is continued for one (1) hour. At the end of this time thirty-four (34) grams of 95% paraformaldehyde is added, and then thirty-six (36) grams of hydrogen chloride gas is bubbled in slowly beneath the surface of the mixture while the temperature is maintained at 65° to 75° C. Stirring is continued for thirty (30) minutes after the hydrogen chloride has been added, and the temperature is then lowered to about 50° C. The mixture is then placed under partial vacuum until about five hundred (500) grams of benzene has been stripped off.

To the remaining material is then slowly added ninety-five (95) grams of pyridine while maintaining the temperature at 65° to 70° C. Stirring is continued for thirty (30) minutes after the pyridine has been added. The reaction is then complete; and the product when cooled to room temperature is a firm homogeneous paste having a slight odor of pyridine. It is readily dispersible in water at 60° C.

In this example, the preparation of the stearyl amido methyl chloride in situ forms no part of the present invention.

##### B. Treatment of fabric

Forty (40) grams of the product prepared in Example I is dispersed by stirring into two hundred (200) cubic centimeters of water at 65° C. When completely dispersed one hundred fifty-five (155) cubic centimeters of cold water and five (5) grams of sodium acetate are added. A piece of cotton poplin is immersed in this treating bath until thoroughly wetted and then the excess liquid is removed by passing between a pair of squeeze rolls. The cloth is then placed in an oven held at 110° C. until just barely dry. It is then placed in a second oven held at a temperature of 155° to 160° C. for a period of 90 seconds. After this heat treatment the cloth is immersed for a few seconds in an aqueous solution containing 0.1% sodium carbonate and 0.1% sodium lauryl sulfate, at about 40° C., to neutralize residual acidity and remove water-soluble decomposition products. It is then rinsed thoroughly in warm water and dried at 110° to 120° C. After being permitted to regain its normal moisture content the treated cloth is found to

possess a high degree of water repellency. That is due to a water-repellent residue on the fibers of the fabric. After subjecting pieces of this treated fabric to standard dry cleaning and laundering tests, it is found to show only slight loss in water-repellency as compared with the same pieces prior to undergoing these tests.

#### EXAMPLE II

##### A. Preparation of quaternary ammonium compound

Two hundred eighty-three (283) grams of stearamide and two hundred sixty-five (265) grams of octadecane nitrile are mixed with two hundred (200) grams of dioxane and two hundred (200) grams of benzene. The mixture is heated to about 70° C. and stirred until the amide and nitrile are dissolved. The solution is then cooled to about 55° C. and thirty-two (32) grams of 95% paraformaldehyde is added. While stirring vigorously forty-six (46) grams of phosphorus trichloride is slowly added and the temperature allowed to rise to 65° to 75° C. Stirring is continued for 15 minutes after the phosphorus trichloride has been added. The mixture is cooled to about 55° C., then thirty-two (32) grams of 95% paraformaldehyde and forty-six (46) grams of phosphorus trichloride are added and the reaction is continued at 65° to 75° C. for 30 minutes. The mixture is then cooled to 50° to 60° C. and approximately two hundred (200) grams of mixed solvent is distilled off under reduced pressure.

To the remaining material is then slowly added ninety-five (95) grams of pyridine while maintaining the temperature at 65° to 75° C. Stirring is continued for 15 minutes after the pyridine has been added and the mixture is then cooled to room temperature. The final product is a firm homogeneous paste which is readily dispersible in warm water.

##### B. Treatment of fabric

Thirty (30) grams of the product prepared in Example II-A is dispersed by stirring into one hundred fifty (150) cubic centimeters of water at 55° C. When completely dispersed, two hundred seventeen (217) cubic centimeters of cold water and three (3) grams of sodium acetate are added. A piece of spun viscose rayon challis is immersed in this treating bath until thoroughly wetted and then the excess liquid is removed by squeezing. The cloth is then placed in a ventilated oven held at 150° to 160° C. for 4 minutes. It is then immersed for a few seconds in an aqueous solution containing 0.1% sodium carbonate and 0.5% isopropanol, after which it is rinsed thoroughly in warm water and dried at about 110° C. After regaining its normal moisture content the treated cloth is found to possess a high degree of water repellency.

The same procedure is given supra, wherein the fabric was cotton and regenerated cellulose, can be used on wool, silk, cellulose acetate, and the various other synthetic fibers.

It is understood that the details set forth in the above examples of treating textile materials may be varied within wide limits without departing from the spirit of this invention as defined in the appended claims.

In the claims the term "formaldehyde" shall be understood as covering gaseous formaldehyde, paraformaldehyde or any other compounds which yield formaldehyde in chemical reactions. Where the term "hydrogen chloride" appears in the claims, it will be understood as covering it per se or any other compounds which yield hydrogen chloride or in chemical reactions under the conditions used in the present process.

We claim:

1. The process of treating textile materials to impart thereto permanent water-repellent properties, which comprises impregnating the same with an aqueous dispersion of a quaternary ammonium compound until the textile material is substantially thoroughly wetted, squeezing out

excess liquid, then subjecting this squeezed material to heat treatment in the absence of added moisture and increasing the temperature after it is dry to between about 150° C. and 230° C., in which step the quaternary ammonium compound is decomposed and hydrochloric acid released and a water-repellent residue left on the textile material, the said water-dispersible quaternary ammonium compound being prepared by the steps which comprise reacting 1 mol equivalent of a chloromethyl acid amide of the general formula



15 wherein R designates a saturated aliphatic hydrocarbon radical of 9 to 21 carbon atoms inclusive and X stands for chlorine, with approximately 0.5-1.5 mols of a straight chain alkyl nitrile containing 10 to 22 carbon atoms inclusive, then reacting this intermediate product with approximately 0.5-1.5 mol equivalents of formaldehyde and approximately 0.5-1.5 mol equivalents of hydrogen chloride to form a second intermediate product, the temperature of reaction in forming these aforesaid 20 intermediate products being substantially 60° to 75° C. inclusive, and thereafter reacting this latter product at temperatures 50° to 75° C. inclusive with 0.5-1.5 mol equivalents of a tertiary amine from the group consisting of pyridine and the C-alkyl substituted pyridines the 25 alkyl group of which does not contain more than 3 carbon atoms.

2. The process of treating textile materials to impart thereto permanent water-repellent properties, which comprises impregnating the same with an aqueous dispersion of a quaternary ammonium compound until the textile material is substantially thoroughly wetted, squeezing out excess liquid, then subjecting this squeezed material to heat treatment in the absence of added moisture and increasing the temperature after it is dry to between about 150° C. and 230° C., in which step the quaternary ammonium compound is decomposed and hydrochloric acid released and a water-repellent residue left on the textile material, the said water-dispersible quaternary ammonium compound being prepared by the steps which comprise reacting 1 mol equivalent of a chloromethyl acid amide of the general formula



30 wherein R designates a saturated aliphatic hydrocarbon radical of 9 to 21 carbon atoms inclusive, and X stands for chlorine with approximately 0.5 to 1.5 mols of a straight chain alkyl nitrile containing not less than 16 carbon atoms but not over 22 carbon atoms, then reacting this intermediate product with approximately 0.5 to 1.5 mol equivalents of formaldehyde and approximately 0.5 to 1.5 mol equivalents of hydrogen chloride to form a second intermediate, the temperature of reaction in forming these aforesaid intermediate products being substantially 60° to 75° C. inclusive, and thereafter reacting this latter product at temperatures of substantially 50° to 75° C. inclusive with a tertiary amine from the group consisting of pyridine and C-alkyl substituted 35 pyridines the alkyl group of which does not contain more than 3 carbon atoms.

3. The process of treating textile materials to impart thereto permanent water-repellent properties, which comprises impregnating the same with an aqueous dispersion of a quaternary ammonium compound and the water-soluble, alkaline reacting salt of a strong base with a weak acid held at a temperature not above substantially 50° C. to avoid premature decomposition of said treating agent, and after the textile material is substantially 40 thoroughly wetted, squeezing out excess liquid, then sub-

jecting this squeezed material to heat treatment in the absence of added moisture and increasing the temperature after it is dry to about 150° C. and 230° C., the time varying inversely with the temperature, in which step the quaternary ammonium compound is decomposed and a water-repellent residue left on the textile material, the amount of the quaternary ammonium compound which is deposited on the textile material in the said impregnation step being 1.0 to 4.0%, this said last mentioned compound being prepared by the steps which comprise reacting 1 mol equivalent of a chloromethyl acid amide of the general formula



wherein R designates a saturated aliphatic hydrocarbon radical of at least 9 to 21 carbon atoms inclusive, and X stands for chlorine with approximately 0.5 to 1.5 mols of a straight chain alkyl nitrile containing not less than 16 carbon atoms but not over 22 carbon atoms, then reacting this intermediate product with approximately 0.5 to 1.5 mol equivalents of formaldehyde and approximately 0.5 to 1.5 mol equivalents of hydrogen chloride to form a second intermediate, the temperature of reaction in forming these aforesaid intermediate products being substantially 60° to 75° C. inclusive, and thereafter reacting this latter product temperatures of substantially 50° to 75° C. inclusive with a tertiary amine from the group consisting of pyridine and C-alkyl substituted pyridines the alkyl group of which does not contain more than 3 carbon atoms.

4. The process of treating textile materials to impart thereto permanent water-repellent properties, which comprises impregnating the same with an aqueous dispersion of a quaternary ammonium compound and a water-soluble alkaline reacting alkali metal salt of a weak acid held at a temperature not above substantially 50° C. to avoid premature decomposition of said treating agent, and after the textile material is substantially thoroughly wetted squeezing out excess liquid, then subjecting this squeezed material to a temperature slightly above the boiling point of water until barely dry, then to an oven temperature of about 150° C. for about two minutes to 230° C. for about 30 seconds, in which heating operation the quaternary ammonium compound is decomposed and a water-repellent residue left on the textile material, the amount of the quaternary ammonium compound which is deposited on the textile material in the said impregnation step being 1.0 to 4.0%, this last mentioned compound being prepared by the steps which comprise reacting 1 mol equivalent of chloromethyl stearamide with approximately 0.5 to 1.5 mol equivalents of stearonitrile, then reacting this intermediate product with approximately 0.5 to 1.5 mol equivalents of paraformaldehyde and approximately 0.5 to 1.5 mol equivalents of hydrogen chloride gas, the reactions being carried out at substantially 60° to 75° C. inclusive and in the presence of a volatile organic solvent for the reactants and with good agitation, removing the major portion of the solvent and thereafter thoroughly mixing pyridine with the second intermediate product and reacting therewith at temperatures of substantially 50° to 75° C. inclusive until the reaction is substantially complete and a mass which is pasty on cooling is secured the alkyl group of which does not contain more than 3 carbon atoms.

5. The process of treating textile materials to impart thereto permanent water-repellent properties, which comprises impregnating the same with an aqueous dispersion of a quaternary ammonium compound and a water-soluble alkaline reacting alkali metal salt of a weak acid held at a temperature not above substantially 50° C. to avoid premature decomposition of said treating agent, and after the textile material is substantially thoroughly wetted

5 squeezing out excess liquid, then subjecting this squeezed material to a temperature slightly above the boiling point of water until barely dry, then to an oven temperature of about 150° C. for about two minutes to 230° C. for about 30 seconds, in which heating operation the quaternary ammonium compound is decomposed and a water-repellent residue left on the textile material, the amount of the quaternary ammonium compound which is deposited on the textile material in the said impregnation step being 10 1.0 to 4.0%, this last mentioned compound being prepared by the steps which comprise reacting 1 mol equivalent of stearamide, approximately 0.5-1.5 mol equivalents of octadecane nitrile, and approximately 1.5-2.5 mol equivalents of paraformaldehyde in the presence of approximately 0.5-0.85 mol equivalents of a phosphorus chloride, at temperatures of substantially 60° to 75° C., inclusive, and under good agitation while the organic reactants are dissolved in a volatile organic solvent therefor, then removing much of the solvent, and adding and reacting approximately 0.5-1.5 mol equivalents of pyridine with this product while continuing to stir and to react at temperatures of approximately 50° to 75° C., inclusive until a firm homogeneous paste product upon cooling is secured, the steps of reaction to secure the quaternary ammonium compound being characterized by the application of heat.

20 6. The process of treating textile materials to impart permanent water-repellent properties, which comprises impregnating the same with an aqueous dispersion of a quaternary ammonium compound and a water-soluble alkaline neutralizing agent until the textile material is substantially wetted, squeezing out excess liquid, then subjecting this squeezed material to heat treatment in the absence of added moisture and increasing the temperature after it is dry to between 150° C. and 230° C., the time varying inversely with the temperature, in which step the quaternary ammonium compound is decomposed and a water repellent residue left on the textile material, the amount of the quaternary ammonium compound which is deposited on the textile material in the impregnation step being about 1.0 to 4.0%, this said last mentioned compound being prepared by the steps which comprise reacting a chloromethyl acid amide of the general formula



30 50 wherein R designates a saturated aliphatic hydrocarbon radical of at least 15 carbon atoms but not over 21 carbon atoms, and X stands for chlorine, with a straight chain alkyl nitrile containing not less than 16 carbon atoms but not over 22 carbon atoms, then reacting this intermediate product with formaldehyde and hydrogen chloride to form a second intermediate, the temperature of reaction in forming these aforesaid intermediate products being substantially 60° to 75° C. inclusive, and thereafter reacting this latter product at temperatures of substantially 50° to 75° C. inclusive with a tertiary amine from the group consisting of pyridine and C-alkyl substituted pyridines, the alkyl group of which does not contain more than 3 carbon atoms, reactants being 1 mol equivalent of the chloromethyl acid amides to substantially 0.5-1.5 mol equivalents of each of the other reactants.

60 65 70 75 7. The process of treating textile materials to impart permanent water-repellent properties, which comprises impregnating the same with an aqueous dispersion of a quaternary ammonium compound and a water-soluble alkaline neutralizing agent until the textile material is substantially wetted, squeezing out excess liquid, then subjecting this squeezed material to heat treatment in the absence of added moisture and increasing the temperature after it is dry to between 150° C. and 230° C., the time varying inversely with the temperature, in which step the quaternary ammonium compound is decomposed

and a water repellent residue left on the textile material, the amount of the quaternary ammonium compound which is deposited on the textile material in the impregnation step being about 1.0 to 4.0%, this said last mentioned compound being prepared by the steps which comprise reacting one mol equivalent of a chloromethyl acid amide of the general formula



wherein R designates an aliphatic hydrocarbon radical 9-21 carbon atoms inclusive, and X stands for chlorine, with approximately 0.5-1.5 mol equivalents of a straight chain alkyl nitrile containing 9-21 carbon atoms inclusive, then reacting this intermediate product with approximately 0.5-1.5 mol equivalents of hydrogen chloride to form a second intermediate product, the temperature of reaction in forming these intermediate products being substantially 60° to 75° C. inclusive, thereafter reacting this latter product at temperatures of substantially 50° to 75° C. inclusive with substantially 0.5-1.5 mol equivalents of a tertiary amine from the group consisting of pyridine and the C-alkyl substituted pyridines, the alkyl group of which does not contain more than 3 carbon atoms, reactants being 1 mol of the chloromethyl acid amides to substantially 0.5-1.5 mol equivalents of each of the other reactants.

8. The process of treating textile materials to impart permanent water-repellent properties, which comprises impregnating the same with an aqueous dispersion of a quaternary ammonium compound and a water-soluble alkaline neutralizing agent until the textile material is substantially wetted, squeezing out excess liquid, then subjecting this squeezed material to heat treatment in the absence of added moisture and increasing the tempera-

ture after it is dry to between 150° C. and 230° C., the time varying inversely with the temperature, in which step the quaternary ammonium compound is decomposed and a water repellent residue left on the textile material, the amount of the quaternary ammonium compound which is deposited on the textile material in the impregnation step being about 1.0 to 4.0%, this said last mentioned compound being prepared by the steps which comprise reacting one mol equivalent of a chloromethyl acid amide of the general formula



15 wherein R designates an aliphatic hydrocarbon radical 9-21 carbon atoms inclusive, and X stands for chlorine, with approximately 0.5-1.5 mol equivalents of a straight chain alkyl nitrile containing 9-21 carbon atoms inclusive, then reacting this intermediate product with approximately 0.5-1.5 mol equivalents of hydrogen chloride to form a second intermediate product, these two reaction steps being carried out at substantially 60° to 75° C. inclusive under good agitation in the presence of a volatile organic solvent for the reactants followed by removal of the major portion of the solvent, thereafter reacting this second intermediate product at temperatures of substantially 50° to 75° C. inclusive with substantially 0.5-1.5 mol equivalents of a tertiary amine from the group consisting of pyridine and the C-alkyl substituted pyridines.

References Cited in the file of this patent

UNITED STATES PATENTS

- |                 |                     |               |
|-----------------|---------------------|---------------|
| 2,250,930       | Evans et al. -----  | July 29, 1941 |
| FOREIGN PATENTS |                     |               |
| 477,991         | Great Britain ----- | Jan. 10, 1938 |